

Patented Dec. 6, 1927.

1,652,078

# UNITED STATES PATENT OFFICE.

GEORG WELTER, OF FRANKFORT-ON-THE-MAIN, GERMANY, ASSIGNOR, BY MESNE ASSIGNMENTS, TO ALLIED PROCESS CORPORATION, OF NEW YORK, N. Y., A CORPORATION OF NEW YORK.

## LEAD-ALKALI METAL CONTAINING BEARING-METAL ALLOYS.

No Drawing. Application filed July 13, 1925, Serial No. 43,393, and in Germany July 24, 1924.

In a prior application, Serial Number 13,633, filed March 6, 1925, there are described bearing-metal alloys consisting essentially of lead with additions of lithium in combination with one or more other alkali metals such as sodium or potassium, or sodium and potassium, each alkali metal in quantity not exceeding about 1% of the alloy. Such alloys possess valuable bearing-metal properties with respect to, for instance, hardness or rigidity, resistivity to shocks, casting qualities, melting point, compression strength, sliding or friction characteristics, and particularly, as compared with previously known lead-bearing metal alloys containing alkali metal and alkaline earth metal additions, a high resistivity against corrosion.

The present invention is an improvement upon that described in said prior application and resides in the discovery that the lithium content of such lead bearing-metal alloys may be reduced to only a proper fraction of 0.1% and the sodium and potassium content to less than 0.5% with a corresponding increase in the resistivity of the alloys against corrosion, while at the same time preserving or even improving the mechanical bearing-metal properties referred to.

*Example 1.*—An alloy containing 0.05% of lithium, 0.3% of sodium and the remainder principally lead has a resistivity to shock of 12 to 13 kg. per mm.<sup>2</sup> and a hardness of 35 kg. per mm.<sup>2</sup>. In a corrosion test consisting of contacting the alloy with steam for a period of ten days, the corrosion produced was smaller than with soft lead.

It is known that the properties of bearing-metal alloys consisting essentially of lead and containing alkali metals are improved by additions of alkaline earth metals. According to the present invention it has been found that the quantity of alkaline earth metal addition necessary to produce the usual effects of such additions may be far below that heretofore employed and regarded as necessary in the production of lead bearing-metal alloys. The improvement of the properties of the alloys of the present invention by alkaline earth metal additions is most favorable when the additions amount to not more than 0.5%.

*Example 2.*—An alloy containing 0.05% of lithium, 0.3% of sodium and 0.4% of cal-

cium and the remainder principally lead, 55 has a resistivity to shock of 14 to 15 kg. per mm.<sup>2</sup> and a hardness of 40 kg. per mm.<sup>2</sup>, and also possesses excellent casting and sliding properties. Its melting point lies in the neighborhood of 350° and the bearing 60 temperature under a load of 4.8 tons rises to, for example, only about 55°. In a corrosion test consisting of contacting the alloy with steam for a period of ten days, the corrosion produced was of scarcely measurable 65 depth.

The alloys can, according to the purpose for which they are designed and the special properties desired, contain the customary additions of copper, nickel, cobalt, zinc, 70 magnesium, bismuth, cadmium, arsenic, antimony, tin, aluminum, silicon and selenium, as well as phosphorus and sulfur. The quantities of such addition agents must however not be so large as to reduce the action 75 of the essential alloying agents.

*Example 3.*—An alloy containing 0.03% of lithium, 0.4% of sodium and 0.5% of calcium and 0.1% aluminum and 0.05% silicon (or 0.2% copper or 0.5% nickel etc.) and the 80 remainder principally lead has a resistivity to shock of 16 to 18 kg. per mm.<sup>2</sup> and a hardness of 40 to 45 kg. per mm.<sup>2</sup>. In a corrosion test consisting of contacting the alloy with steam for a period of ten days, the 85 corrosion produced was similar to that of soft lead.

The sodium additions of the foregoing examples may be substituted by equal amounts of potassium or supplemented by 90 additions of potassium in quantity preferably not exceeding about 0.1%.

The alloys of the present invention may be made in the usual way, for example, by melting the ingredients together preferably using preliminary alloys of the alkali and alkaline earth metal additions such as alloys of sodium and lithium, lithium and potassium, or sodium, potassium and lithium. Other methods of forming the alloys, 100 for instance, by electrolysis, diffusion, compressing powders of the ingredients, etc., may also be employed.

## Claims:—

1. Bearing metal alloys consisting essentially of lead and comprising lithium in quantity sufficient to produce an appreciable hardening effect but not in excess of about 105

0.05% and an appreciable amount of at least one other alkali metal not substantially in excess of about 0.5%.

2. Bearing metal alloys consisting essentially of lead and comprising lithium in quantity sufficient to produce an appreciable hardening effect but not in excess of about 0.05% and an appreciable amount of sodium not substantially in excess of about 0.5%.

10 3. Bearing metal alloys consisting essentially of lead and comprising lithium in quantity sufficient to produce an appreciable hardening effect but not in excess of about 0.05%, an appreciable amount of sodium not substantially in excess of about 0.5%, and an appreciable amount of potassium not substantially in excess of about 0.1%.

20 4. Bearing metal alloys consisting essentially of lead and comprising lithium in quantity sufficient to produce an appreciable hardening effect but not in excess of about 0.05%, an appreciable amount of at least one other alkali metal not substantially in excess of about 0.5%, and an appreciable amount of an alkaline earth metal not substantially in excess of about 0.5%.

25 5. Bearing metal alloys consisting essentially of lead and comprising lithium in quantity sufficient to produce an appreciable

hardening effect but not in excess of about 30 0.05%, an appreciable amount of sodium not substantially in excess of about 0.5%, and an appreciable amount of an alkaline earth metal not substantially in excess of about 0.5%.

35 6. Bearing metal alloys consisting essentially of lead and comprising lithium in quantity sufficient to produce an appreciable hardening effect but not in excess of about 0.05%, an appreciable amount of sodium not substantially in excess of about 0.5%, an appreciable amount of potassium not substantially in excess of about 0.1%, and an appreciable amount of an alkaline earth metal not substantially in excess of about 0.5%.

40 7. Bearing metal alloys consisting essentially of lead and comprising lithium in quantity sufficient to produce an appreciable hardening effect but not in excess of about 0.05%, an appreciable amount of sodium not substantially in excess of about 0.5%, an appreciable amount of potassium not substantially in excess of about 0.1%, and an appreciable amount of calcium not substantially in excess of about 0.5%.

45 In testimony whereof, I affix my signature.

50 GEORG WELTER.